

May 11, 1937.

H. GORDON

2,079,706

METHOD OF LAYING CHANNEL FLAPS

Filed Nov. 8, 1934



*Fig. 1.*



*Fig. 2.*



*Fig. 3.*



*Fig. 4.*

Inventor  
*Hiram Gordon*

By  
*W. S. Howell*

Attorney

## UNITED STATES PATENT OFFICE

2,079,706

## METHOD OF LAYING CHANNEL FLAPS

Hiram Gordon, Columbus, Ohio, assignor to The  
Walker T. Dickerson Company, Columbus,  
Ohio, a corporation of Ohio

Application November 8, 1934, Serial No. 752,087

7 Claims. (Cl. 12—142)

This invention relates to improvements in footwear, and has particular reference to shoes of the type wherein the outsoles are marginally stitched in secured relationship with shoe welts or uppers.

In shoes of the type embodying stitched outsoles, it is customary to conceal the stitching, when the outsoles are viewed from the bottom, by the provision of channel strips or flaps. In the manufacture of such shoes, it is the ordinary practice to slit the outsoles marginally, while the leather comprising such an outsole is in a relatively moist or tempered state, to form the marginal strips or flaps integrally with the outsole. With the flaps in an elevated position, the marginal portions of such outsoles are then stitched to welts connected with the shoe uppers or in the case of other types of shoes directly to said uppers. Following the stitching operation, an adhesive is placed on the contiguous surfaces of the channel strips or flaps and marginal portions of a shoe outsole and following a drying operation, the channel strips are pressed into engagement with the outsoles in order to be adhesively connected therewith in stitch concealing relationship.

Heretofore, the adhesive employed in this operation contains or is composed largely of rubber which requires that the leather comprising the outsole must be in a comparatively dry condition before the rubber containing adhesive will function in the matter of uniting the channel strip to the outsole. Furthermore, it is a matter of common knowledge that a channel strip secured by the usual process after a short period of wear will become disengaged from the adjoining surfaces of the outsole so that it presents a rough, uneven and undesired appearance and, moreover, leaves the stitching of the outsole directly exposed to shoe wear.

In accordance with the present invention, use is made of a pyroxylin base cement which has the capability of uniting leather surfaces when the leather is in a moist or tempered state so that through the employment of the pyroxylin base cement, I am enabled to apply the same to an outsole immediately following the sewing of the outsole in connection with the shoe upper and to cause the leather surfaces united by said cement to maintain their adhesion under prolonged periods of use and service, to the end of expediting and facilitating the laying of channel strips on the sewed outsoles of shoes and to improve the wearing qualities of such shoes by preventing separation of the channel strips from

the outsoles when the shoes are placed in wear and service.

The present invention constitutes a continuation-in-part of my prior application, Serial No. 678,802 filed July 3, 1933, and is particularly directed to a shoe formed in accordance with the process set forth in my aforesaid application.

For a further understanding of the invention, reference is to be had to the following description and the accompanying drawing, wherein:

Fig. 1 is a perspective view showing a welted shoe as contained on a last and in process of manufacture, the skived channel strip of the outsole being shown in an elevated position admitting of the stitching of the outsole to the adjoining welt of the shoe and providing for the application of a cement thereto;

Fig. 2 is a transverse sectional view taken through a welted shoe constructed in accordance with the present invention;

Fig. 3 is a view in side elevation, partly in vertical section, disclosing the shoe in a press in which the channel strip is forced into engagement with the outsole;

Fig. 4 is an enlarged longitudinal sectional view taken through the stitching employed in uniting the outsole with the welt strip.

Referring more particularly to the drawing, the numeral 1 designates the outsole of a welted shoe, although it will be understood that the invention may be employed in the manufacture of any type of shoe wherein a channel outsole is provided. In the process of manufacturing a welt shoe, the insole is skived or cut to produce a depending marginal flange 2. To this flange 30 there is secured the lower portions of the shoe upper 3 together with the welt 4. The welt usually comprises a strip of leather which surrounds the flange 2, and is fastened to the adjoining portions of the upper and the flange 2 by means of a fine wire stitching or lacing 5. The outsole 1, which is composed of leather, and in a moist or tempered state, is then placed over the insole in engagement with the flange 2 and the welt 4, leaving a space 7 between the bottom of the insole and the upper surface of the outsole bounded by the flange 2, this space being ordinarily filled with a composition material such as ground cork and a binder. The outsole is then secured by means of the stitching indicated at 8 to the welt 4, the stitching being effected through the marginal edges of the outsole as shown in Fig. 2.

In order to protect and conceal the stitching 8, the outsole of such a shoe is horizontally slit

contiguous to its lower and marginal outer edges, while the leather of the outsole is in a moist or tempered state facilitating such an operation, to form an integral marginal flap 9 known in the 5 industry as a channel strip. This strip, after the stitching 8 has been effected, is adapted to be pressed downwardly into flush position with the bottom of the outsole and retained in this position, covering the outsole stitching, by the 10 use of a suitable cement. As previously stated, the strip 9 due to prior methods and means for cementing the same, tends to readily disengage itself from the outsole after a short period of use or wear, so that when the shoe is viewed from 15 the bottom or from the side, the loosened strip presents an unfinished and unsightly appearance which mars the appearance of such a shoe and in addition exposes the stitching 8 to direct wear.

The stitching 8 usually comprises looped 20 threads 10, as shown in Fig. 4, which pass through registering awl and needle openings 11 formed in the welt 4 and the outsole, while a bobbin thread 12 passes through the lower loops 10 and is normally positioned between the body of 25 the outsole and the upper surface of the channel strip 9, the stitching being protected by the channel strip. Thus when the channel strip becomes loosened, the bobbin thread 12 is exposed to direct wear and to the elements, causing deterioration 30 and breakage thereof so that the union between the outsole and the welt sole is weakened with accompanying premature destruction of the shoe. It is therefore very important that the channel strip should be continuously maintained in its 35 flush position with the outsole and in secured relationship therewith not only from a standpoint of appearance but to preserve the mechanical efficiency and prolong the life of a shoe employing an outsole attached by stitching.

40 In manufacturing a shoe comprising the present invention, following the channeling of a leather outsole, while the latter is in a moist or tempered state, to produce the strip 9 and the subsequent stitching, as at 8, of the outsole to the 45 welt, a pyroxylin base cement is applied by brush or otherwise, to the adjoining surfaces of the channel strip and the outsole. I have found that a pyroxylin base cement having substantially the 50 composition set forth hereinafter, may be applied to the outsole when the latter is in substantially the same state of temper or moisture as when slit or stitched. In other words, there is no 55 period of drying of the outsole following the stitching thereof required in order to render the adhesive effective.

Immediately following the application of the 60 pyroxylin base cement to the channel strip and outsole, the lasted shoe is transferred to a press which may be of the type disclosed in Fig. 3. In this press, the lasted shoe is placed with its 65 outsole engaging with a resilient pad 13 and the entire outsole subjected to a pressure in excess of approximately 12 pounds per square inch which is applied simultaneously over the entire 70 area of the channel strip. By the employment of these high pressures, the pyroxylin base cement adhesively unites the channel strip with the adjoining portions of the outsole in overlapping and protecting relationship with respect to the 75 stitching 8 and, moreover, the cement is forced into the needle or awl openings through which the stitching 8 passes, whereby to surround, protect and lock the threads with the cement. By filling these openings with cement, there is produced in said openings upon the hardening and

setting of the cement, pegs or pins of the cementitious material which of themselves serve in a manner substantially independently of the stitching to firmly unite the outsole and welt in fixed relationship.

5 As a satisfactory non-rubber cement, I have found a mixture composed of the following ingredients to impart good results, although it should be understood that I reserve the right to employ other pyroxylin base cements having 10 equivalent penetrating, adhesive and flow properties.

|         | Per cent by weight | Per cent              |
|---------|--------------------|-----------------------|
| Solvent | 88.6               | Toluol 40.9           |
|         |                    | Butyl acetate 17.6 15 |
|         |                    | Alcohol 30.1          |
| Solids  | 11.4               | Nitrated cotton 7.4   |
|         |                    | Resin 3.0             |
|         |                    | Plasticizer 1.0       |

20 By means of the present invention, I am enabled to produce a channeled outsole wherein looseness of the channel strip upon wear or use of the shoe is prevented, and whereby union is effected of such a character that irrespective 25 of wear, the channel strip will maintain its adhesion relationship with the adjoining portions of the outsole. Due to this fact, the outsole stitching is protected, yet the customary unsightly appearance of a shoe after initial wear is avoided. Also, economies are obtained in the 30 actual manufacture of a shoe in accordance with my invention due to avoidance of delay heretofore present in the drying of leather and of the rubber cements of conventional composition.

35 The pyroxylin base cement comprising the present invention possesses a neutral color when applied to leather, so that it does not stain or dis-color the leather in any way or effect its natural appearance. The invention is applicable to any type of shoe having a stitched channeled outsole and while it is of particular importance in the manufacture of welted shoes, it is also of corresponding importance in the manufacture of 40 shoes of the "McKay" or "Littleway" types in which the outsoles are channeled and stitched directly to the insole and shoe upper without 45 using a welt.

What is claimed is:

1. As a new article of manufacture, a shoe having a stitched channeled outsole with the flap 50 thereof permanently united to the sole margin under ordinary conditions of wear and service with a pyroxylin cement composed approximately of toluol 40.9%, butyl acetate 17.6%, alcohol 30.1%, nitrated cotton 7.4%, resin 3.0% and plasticizer 1.0%.

55 2. In the manufacture of shoes having sewed outsoles, the steps which comprise tempering an outsole, slitting the outsole inwardly and horizontally around its marginal edges to produce an integral and flexible channel flap, stitching the outsole marginally and independently of the flap to secure the outsole to the adjoining upper portions of a shoe, substantially immediately applying to the adjoining portions of the flap and outsole with the leather of the outsole in the 60 same condition of temper as when cut and sewed, a pyroxylin cement effective in the presence of moisture, substantially immediately smoothing the flap into place on said sole to conceal the 65 marginal stitching thereof, and subjecting said outsole to pressure simultaneously over substantially the full area of said flap to permanently bond said flap in unbroken engagement with the outsole.

70 3. In the manufacture of shoes having sewed 75

outsoles, the steps which comprise tempering an outsole, slitting the outsole inwardly and horizontally around its marginal edges to produce an integral and flexible channel flap, stitching the outsole marginally and independently of the flap to secure the outsole to the adjoining upper portions of a shoe, substantially immediately applying to the adjoining portions of the flap and outsole with the leather of the outsole in the same condition of temper as when cut and sewed, a pyroxylin cement effective in the presence of moisture, substantially immediately smoothing the flap into place on said sole to conceal the marginal stitching thereof, and subjecting said flap to sufficient pressure to permanently bond said flap in unbroken engagement with the outsole.

4. In the manufacture of shoes having channeled outsoles wherein the channel flaps are adhesively secured to the marginal portions of the shoe outsoles to conceal stitching, the steps which comprise applying a pyroxylin cement effective in the presence of moisture between the channel flap and outsole while the same are in a condition of temper and applying pressure over substantially the full area of said flap to bond the same to the outsole.

5. In the manufacture of shoes having sewed outsoles, the steps which comprise tempering an outsole, slitting the outsole inwardly and hori-

zontally around its marginal edges to produce an integral and flexible channel flap, stitching the outsole marginally and independently of the flap to secure the outsole to the adjoining upper portions of the shoe, substantially immediately applying a pyroxylin cement effective in the presence of moisture to the adjoining portions of the flap and outsole with the leather of the outsole in the same condition of temper as when cut and sewed, substantially immediately smoothing the flap into place directly on said outsole to conceal the marginal stitching thereof, and subjecting said flap to sufficient pressure to permanently bond said flap in unbroken engagement with the outsole, there being no intervening material between said flap and said outsole except said cement.

6. The process of cementing leather surfaces together while in a moist or tempered condition which comprises the steps of applying between said surfaces a pyroxylin cement effective in the presence of moisture and then joining said surfaces.

7. In the laying of channel flaps in shoes, the steps of applying a pyroxylin cement effective in the presence of moisture to said flap while the same is in a condition of temper, and then joining the flap to a shoe outsole.

HIRAM GORDON. 30